

Aug. 14, 1928.

1,680,705

E. THOMSON

METHOD OF MAKING INSULATORS

Filed Nov. 29, 1922



Inventor,  
Elihu Thomson,  
by Alexander S. Hunt,  
His Attorney.

## UNITED STATES PATENT OFFICE.

ELIHU THOMSON, OF SWAMPSCOTT, MASSACHUSETTS, ASSIGNOR TO GENERAL ELECTRIC COMPANY, A CORPORATION OF NEW YORK.

## METHOD OF MAKING INSULATORS.

Application filed November 29, 1922. Serial No. 604,075.

The present invention relates to electrical insulators and more especially to strain insulators, and the object of the invention is to provide an improved method of connecting the metal parts to the insulative parts.

During recent years and especially since the introduction of the suspension system of supporting high potential electric lines, the majority of strain insulators used have been of the cemented cap and pin type, that is to say, the insulative member of porcelain has a cup-shaped part, to the outside of which a metal cap is cemented and to the inside of which a metal pin or bolt is cemented.

After a cemented strain insulator has been in use two or three years, there develops a very pronounced tendency to fail by breakage of the porcelain and this failure has been generally attributed to the progressive hydration of the cement and the unequal coefficients of expansion possessed by the closely united metallic and non-metallic parts. Many attempts have been made to provide a satisfactory mechanical connection between the parts of strain insulators in an endeavor to avoid the practical defects of the cemented insulators, but none of them up to the present time have been effective in displacing that type to a material degree, for they either require the porcelain to be made in such complex shapes that a uniformly satisfactory product is rendered difficult of accomplishment or else the mechanical connection parts work loose or the porcelain part breaks by reason of the bearing of the metal parts thereon being localized instead of distributed as in the case of the cemented type.

In carrying out my invention, I employ a vitreous insulative member of the cap and pin type having a bore or opening with an enlargement to provide an internal shoulder and cast or mold the metal pin or bolt therein which, upon cooling, shrinks away from the insulator wall slightly but sufficient to permit each material to expand and contract independently of the other while the bearing of the one on the other is uniformly distributed, and the cap part is cast or separately fitted about the outside of the insulator.

On account of the relatively high coefficients of expansion possessed by porcelain or other vitreous materials commonly used in insulators, it is impractical to pour molten

metal onto or into them without breakage. Moreover, by reason of the great stresses imposed upon strain insulators in use, it is highly desirable that the hardware be of a strong hard metal, such as iron or an alloy thereof, the melting point of which is higher than that of the usual insulating substances.

I have found that insulators of fused quartz have such a low coefficient of expansion and extremely high melting point that molten iron or iron alloy can be poured into a cavity therein without injury to the insulator and that it is also practical to insert a bar of iron or steel into the cavity of a quartz insulator and bring it to a molten condition therein by application of heat to the exterior of the quartz insulator without injury to the latter.

In the accompanying drawing, I have indicated the simplest embodiment of my invention and certain steps by which it is made. Fig. 1 is an axial section of the strain insulator; Figs. 2 and 3 are axial sections of the fused quartz insulator showing how a metal bolt or pin is cast therein; Figs. 4 and 5 are similar views showing how an iron bar is molded at its lower end to fill the cavity of the insulator; and Figs. 6 and 7 indicate separate steps in the formation of a quartz insulator member.

As indicated in Fig. 1, the insulating member 1 of fused quartz has a hollow globular head 2 having an internal shoulder and a tubular stem 3 within which a bolt 4 with an expanded head 5 is located, while the outside of the globular head 2 is received between an annular seat plate 6 and a supporting yoke 7 held together by rivets or bolts. The free ends of the yoke 7 and the bolt 4 are provided with suitable means such as eyes or threads for attachment of the insulator to the stress applying device.

To cast a bolt 4 in a quartz insulating member 1, the latter is positioned with head down and the stem lengthened in effect by a detachable extension cylinder 9 and the entire cavity filled with molten metal. The extension cylinder 9 is removed after the metal is cooled so as to expose a corresponding length of the bolt beyond the end of the insulating member 1, in which a thread 10 may be cut.

To upset or mold the end of a plain iron bar within the quartz insulating member, a bar with excess length is introduced within

the hollow of the insulating member, as indicated in Fig. 4, and heat applied to the outside of the head 2 of the latter until it is raised to a sufficiently high temperature to 5 soften or melt the end of the contained bar which then settles until the hollow of the head 2 is filled with metal, as indicated in Fig. 5.

Upon allowing to cool, the cast or molded 10 metal shrinks away from the wall of the insulator sufficiently to upset any tendency to adhere thereto.

While the insulating member 1 may be made in various shapes, the plain one shown 15 is very satisfactory in service and can be manufactured of fused quartz very economically. I make a carbon core 11 approximately the same size as the pin or bolt 4, connect its ends to metallic electric conductors, embed it in quartz grains, and raise the 20 temperature thereof to the fusion point of quartz by passing a strong electric current through it for a sufficient period of time to produce an encrustation of quartz thereabout 25 of the desired thickness. When the fused quartz encrustation or shell is cooled or practically cooled, it is removed from the bed of quartz grains and has the appearance indicated in Fig. 6. The carbon core 11 is re-

30 moved, as by drilling, and the hollow head 2 formed thereon by local heating and sealing the end of the shell, as indicated by the dotted lines 12 in Fig. 7, and expanding it by air pressure similar to the method of blowing glass bulbs.

35 In case it is desired to provide petticoats or other projections on the insulating member 1, they are separately formed and then homogeneously united at any desired point thereon by fusion.

40 Although I have shown and described only one embodiment of the invention, I do not desire to be restricted thereto.

45 What I claim as new and desire to secure by Letters Patent of the United States, is,—

1. The method of making electric insulators comprising the forming of an insulating member of fused quartz with a bore and forming therein by fusion a metallic pin.

50 2. The method of making electric strain insulators comprising the forming of an insulating member of fused quartz with a bore therein enlarged to provide an internal shoulder, and forming in said bore a metallic tension member.

55 In witness whereof, I have hereunto set my hand this 24th day of November, 1922.

ELIHU THOMSON.